

## UNITED STATES PATENT OFFICE

ALEX BROOKING DAVIS, OF CINCINNATI, OHIO, ASSIGNOR TO A. B. DICK COMPANY, OF CHICAGO, ILLINOIS, A CORPORATION OF ILLINOIS

## STENCIL SHEET AND METHOD OF MANUFACTURING THE SAME

No Drawing.

Application filed October 26, 1926. Serial No. 144,403.

This application is a continuation of an application filed by me October 7, 1924, for Cellulose ester compositions, Serial No. 742,266.

5 This invention relates to stencil sheets and to a method of manufacturing the same.

The principal object of this invention is to provide a stencil sheet which is readily and easily stencilizable by means of either 10 type or stylus, to present stencil openings which are well opened, clean-cut, and clear, so that the printed impressions produced by the stencil will be well and evenly inked, clean-cut and clear.

15 A further object of this invention is to provide a stencil sheet of the character described which is not expensive or difficult to manufacture, and one which requires for its manufacture only commercially available materials.

20 A further object of this invention is to provide a sheet of the character described which is durable and lasting, being capable of surviving crumpling, creasing and 25 handling without evil effect, and will retain unimpaired over a long period of time its ability to be stencilized or to yield satisfactory printing.

Another object of this invention is to provide 30 a method of manufacturing a stencil sheet of the character referred to, which method tends to yield sheets of the desired quality uniformly, and to provide a method which is suitable for the manufacture and 35 sale on a commercial scale of stencil sheets having the superior characteristics referred to above.

Other objects of this invention will be in part obvious and in part pointed out hereinafter.

40 In accordance with my invention, I utilize in the manufacture of stencil sheets polyhydric alcohol characterized by ununiform esterified condition or character of hydroxyl 45 groups, that is, esterified in an ununiform manner, for instance, as with different substances. I incorporate such a substance in a suitable cellulose colloid dissolved in a suitable solvent to form the stencil sheet 50 coating compound, and then produce the

stencil sheet by coating sheets of suitable base material, such as "yoshino", or other suitable porous, open-weave material, with this compound, and allowing the coated sheets to dry. Stencil sheets produced in accordance with the above will be found to possess softness and flexibility without "tack", and will not be injured by being creased or crumpled, and will be very durable both before and after being stencilized; the coating will be well set, not appreciably hygroscopic, and at the same time will respond readily to stencilizing by either type and stylus, opening up the stencil cuts faithfully and well, and will yield well inked and clear impressions when prints are made with the stencil.

In further illustration of my invention the following examples of methods of making stencil coating compounds are presented:

1. To a mixture of 100 parts of 5% solution of nitrocellulose dissolved in 75% ether—25% alcohol, there may be added 5 parts of propionyl diacetin.

2. To a mixture of 100 parts of 5% solution of nitrocellulose dissolved in 75% ether—25% alcohol, there may be added 5 parts of butyryl diacetin.

Sheets of suitable base material may be 50 coated with either compound. Upon the evaporation of the volatile solvent from either coating it will be found that the glycerol ester has incorporated itself with the nitrocellulose with the effect of endowing 55 the mass with softness and flexibility, and that the sheet will be possessed of the other desirable characteristics mentioned heretofore.

The mono-, di- and tri-acetins formed by 60 esterifying glycerol with acetic acid are already known to be suitable agents for incorporating in plastic pyroxylin masses, but all 65 these substances possess disadvantages for stencil manufacture, in that the monoacetin and diacetin are quite hygroscopic, and even 70 the triacetin possesses some hygroscopicity. When, however, at least one hydroxyl of the 75 glycerol molecule is esterified with a fatty acid of higher molecular weight than acetic, 80

the boiling points are raised, and this in itself constitutes a distinct advantage for stencil sheet manufacture, as the substances are less volatile. As above mentioned, glycerol is a suitable polyhydric alcohol, and when two hydroxyls of the glycerol molecule have been esterified with acetic acid and the third hydroxyl then esterified with an acid of higher molecular weight than acetic acid, compounds are obtained which possess distinct advantages over those substances obtained where all three hydroxyls have been esterified in a uniform manner, as by the use of a single acid, such as acetic acid or formic acid.

Diaceto glycerol propionate may readily be produced by esterifying glycerol with mixtures of acetic and propionic anhydride, or it may be prepared more cheaply by esterifying glycerol by means of acetic anhydride to which has been added a portion of anhydrous or nearly anhydrous propionic acid, both of which substances are obtainable in quantity commercially at the present time. Glycerol esterified in this manner, yielding diaceto glycerol propionate, shows a boiling point for the technically pure substance of 263 to 270 degrees C.—approximately 10 degrees above the boiling point of pure triacetin. Again, glycerol may be esterified with acetic anhydride to which has been added one molecular portion of butyric acid, in which case there is obtained technically pure diaceto glycerol butyrate, and again it is found that the higher molecular weight of the butyric acid raises the boiling point, the technically pure substance boiling at approximately 274 to 278 degrees C. Both of these substances mentioned are less soluble in water and less hygroscopic than triacetin and they maintain this advantage when incorporated in plastic pyroxylin masses or in masses suitable for the formation of films, and, therefore, when used for stencil sheet coatings produce a superior product for the purpose desired. In view of this disclosure it will be evident to those skilled in the art that still higher acids than butyric may be employed to advantage in producing these mixed esters for stencil sheet manufacture. These substances are particularly desirable for incorporation in pyroxylin stencil sheet coatings, since in these a high degree of softness and flexibility is desired. They incorporate perfectly with pyroxylin or other forms of cellulose.

For the specific mixed esters mentioned above, other polyhydric alcohols than glycerine may be used, such for instance as the glycols, and when all the hydroxyl hydrogens have been replaced and the substance rendered anhydrous, they possess the valuable properties of being less hygroscopic, less soluble in water, and having a higher

boiling point than the acetyl derivatives of the parent substance, and, in certain instances, other properties which work to their advantage in the manufacture of cellulose stencil sheets. While in certain types of masses these mixed esters will incorporate themselves in nitrocellulose in proportions of weight for weight. I do not restrict myself to their use in this proportion, since to obtain compositions of definite properties it is desirable to increase or reduce the proportion, which may fall as low as 10 to 1, since even in this small proportion the effect of these mixed esters is readily obvious.

If desired, the softness and flexibility may be still further emphasized when other modifying agents as well are mixed with the pyroxylin solutions as plasticizers. Among such agents, I may mention chlorinated naphthalene and other halogenated aromatic and aliphatic compounds.

What I claim is:

1. A stencil sheet of the character described, comprising base material having a type impervious cellulose compound coating including polyhydric alcohol ununiformly esterified by means of acetic acid and propionic acid.

2. A stencil sheet of the character described, comprising base material having a type impervious cellulose compound coating including glycerol ununiformly esterified by means of anhydrous acetic acid and propionic acid.

3. A stencil sheet of the character described, comprising base material having a coating including cellulose nitrate and diaceto glycerol propionate.

4. A stencil sheet of the character described, comprising base material having a coating including cellulose nitrate and diaceto glycerol propionate, and a halogenated hydrocarbon modifying agent.

5. A stencil sheet of the character described, comprising base material having a coating including cellulose nitrate and ununiformly esterified propionyl acetyl ester of glycerin boiling between 263° and 270° C. at atmospheric pressure.

6. A coating for stencil sheets comprising the mixture of five per cent. solution of nitro-cellulose dissolved in ether-alcohol and propionyl diacetin in the relative ratio of twenty parts of solution to one part propionyl diacetin.

7. A stencil sheet of the character described, comprising base material having a type impervious cellulose compound stencil coating including polyhydric alcohol non-uniformly esterified by organic acids having different molecular weights, one of said acids having a higher molecular weight than formic acid.

8. A stencil sheet of the character de-

scribed comprising base material having a type impessible cellulose compound stencil coating including polyhydric alcohol non-uniformly esterified by different fatty acids 5 one of such acids being acetic acid and another being an acid having higher molecular weight than acetic acid.

9. A stencil sheet of the character described, comprising base material having a type-impessible cellulose compound stencil coating including an ester of a polyhydric alcohol at least two hydroxyl groups of which have been replaced by radicles of different acids, one of which contains at least 10 two carbon atoms.

10. A stencil sheet of the character described comprising base material having a type-impessible cellulose compound stencil coating including an ester of a polyhydric alcohol at least two hydroxyl groups of which have been replaced by radicles of different acids, one of which contains at least 15 three carbon atoms.

This specification signed this 15th day of 25 October, 1926.

ALEX BROOKING DAVIS.

30

35

40

45

50

55

60

65